

# United States Patent

[19]

Backlund

[11] 3,907,631

[45]\*Sept. 23, 1975

[54] **METHOD OF PERFORMING A SURGE-BOIL STEP DURING THE HEATING PERIOD OF A LIGNOCELLULOSIC MATERIAL COOKING STAGE**

[76] Inventor: **Sture Olof Erik Backlund,**  
Sundsvall, Sweden

[\*] Notice: The portion of the term of this patent subsequent to Feb. 19, 1991, has been disclaimed.

[22] Filed: **June 8, 1973**

[21] Appl. No.: **368,032**

## Related U.S. Application Data

[63] Continuation-in-part of Ser. No. 209,883, Dec. 20, 1971, Pat. No. 3,793,137.

## Foreign Application Priority Data

May 14, 1973 Sweden ..... 7306760

[52] U.S. Cl. .... **162/42; 162/61**

[51] Int. Cl.<sup>2</sup> ..... **D21C 7/12**

[58] **Field of Search** ..... 162/42, 61

## [56] References Cited

### UNITED STATES PATENTS

|           |         |                |          |
|-----------|---------|----------------|----------|
| 1,831,206 | 11/1931 | Swanson et al. | 162/61 X |
| 1,905,050 | 4/1933  | Pelot et al.   | 162/61   |
| 3,298,889 | 1/1967  | Laakso         | 162/42 X |
| 3,467,573 | 9/1969  | Vogel          | 162/42 X |

*Primary Examiner*—S. Leon Bashore

*Assistant Examiner*—Arthur L. Corbin

## [57] ABSTRACT

In the periodic cooking of lignocellulosic material in a digester, the homogeneity of the digester contents can be improved by the interposition of at least one surge-boil during the cooking process which is effected by reducing the pressure in the digester together with the direct introduction of steam into the bottom of the digester, simultaneous with pressure reduction, at a rate of at least 0.1 ton steam/minute.

**1 Claim, 2 Drawing Figures**



FIG.2



**METHOD OF PERFORMING A SURGE-BOIL STEP  
DURING THE HEATING PERIOD OF A  
LIGNOCELLULOSIC MATERIAL COOKING  
STAGE**

This application is a continuation-in-part of my co-pending Application Ser. No. 209,883 filed Dec. 20, 1971 now U.S. Pat. No. 3,793,137.

This invention relates to a method of obtaining homogeneous digestion in the periodic cooking of a lignocellulosic material.

In all pulp manufacturing processes uniform cooking is of great importance, with respect both to economy and to the quality of the pulp. The reasons for non-uniform cooking vary with the process type. The Swedish Pat. Spec. No. 345,885 enumerates the most important factors affecting the homogeneity at periodic cooking and it describes a method which has as its object to eliminate the most dominating one of these factors, viz, the cooking liquor circulation.

Experiences from a mill installation prove that the techniques applied according to the method, i.e., surge-boil, has a very positive effect on the homogeneity of the cooking.

It was found, however, that an important factor in conjunction with the surge-boil method was the gassing condition of the digesters, i.e., the overpressure of air and other gases in the digester when the surge-boil commences during the cooking process. An effective degassing of the digesters prior to the surge-boils is one condition for obtaining a full surge-boil effect, i.e., a fully satisfactory digestion uniformity in the digester.

It has proved difficult, however, to carry out a complete degassing of the digesters in time before the surge-boil stage, particularly in the case of rapid heating processes.

When experiments were made for overcoming these difficulties, it was found by surprise that the system could be rendered less sensitive to overpressure at the surge-boils by supplying direct steam to the digester bottom.

The surge-boils, thus, are brought about according to the present invention by pressure reduction in the digester and simultaneous direct supply of steam to the digester bottom. Thereby the surge-boils become more efficient, especially during rapid heating processes. The steam supply is to be substantial, i.e., at least 0.1 ton steam/minute, preferably 0.1 - 0.5 ton steam/minute.

The pressure reduction in the digester bringing about a surge-boil is effected either by degassing from the digester top or by supply of cooling liquor, for example cooking liquor or water, to the digester top.

At least one of said surge-boil steps is carried out during the heating period of the cooking stage at a point of time when the chlorine number of the pulp is 30-20.

The duration of the surge-boil periods may vary, but should be at least 5 seconds. A normal period is 10 seconds - 20 minutes, suitably 1 - 10 minutes and preferably 2 - 5 minutes.

FIG. 1 shows a periodic sulphate digester with a circulation system for indirect heating, and

FIG. 2 shows such a digester with a system for direct heating with steam.

The invention is described in the following by way of two examples with reference to the drawings. Although the examples refer to sulphate cooking, the method acc-

cording to the invention can be applied, for example, to sulphite and bisulphite cooking.

**EXAMPLE 1**

The cooking is carried out in a periodic sulphate digester having a volume of 125 m<sup>3</sup>. The digester is equipped with a circulation system for indirect heating according to FIG. 1. The digester is charged by means of a liquor packing method with about 23 tons of wood chips calculated on the dry basis. White liquor and black liquor are charged in an amount such that the alkali charge is 200 kg active alkali (NaOH) per ton of absolutely dry wood, and the wood:liquor ratio is 1:3.5. The circulation pump 1 is started already whilst the chips are being charged, and it sucks liquor from the digester through a strainer unit 2. The cooking liquor is circulated through the heat-exchanger 3 for heating and is distributed after the heat-exchanger so that 80% of the volume flow is passed to the top of the digester via a conduit 4 and the remaining 20% is passed to the digester bottom via a conduit 5. The liquor circulated to the top of the digester is distributed over the chips by means of centrifugal pressure sprays 6. The heating to 170° C. is effected within 150 minutes by indirect heating with steam in the heat-exchanger 3 and during the surge-boils also by direct heating with steam. The temperature in the top circulation conduit 4 during the heating of the cook having reached 153° C., the first surge-boil is carried out. This is effected in such a manner that the valve 7 is closed automatically by a time clock which was started at the start of the cooking process.

Thirty seconds after the closing of valve 7, the degassing valve 8 is opened whereby the digester is degassed through the conduit 9, and at the same time the steam valve 10 is opened for supplying direct steam through a conduit 11. After 5 minutes the valves 8 and 10 are closed, and the valve 7 is opened.

The heating of the cook can thereafter proceed in a normal way. During said de-gassing and simultaneous steam supply to the digester bottom, a surge-boil takes place in the digester, which owing to the steam supply becomes relatively insensitive to over-pressure in the digester. The same surge-boil step is repeated also at 160° C. and at 167° C. The cook is held at the maximum temperature of 170° C. for about 1 hour. Subsequent to the in-take of about 10 m<sup>3</sup> cooling liquor, the digester is blown. Blowing time = 30 minutes.

The chlorine number of the pulp was 5.7 and the shive content when screening an average sample from the cook in a Wennberg-strainer having a slit width of 0.20 mm was 1.0%. The shive content of a cook, at which the surge-boil technique was not utilized, was 5.2% at a chlorine number of 5.7.

**EXAMPLE 2**

The cooking is carried out in a periodic sulphate digester having a volume of 125 m<sup>3</sup> according to FIG. 2. The digester is equipped for direct heating by steam. The digester is charged with wood chips, which are packed by means of a steam packing unit so that the amount of chips in the digester is about 25 tons of chips calculated on the dry basis. White liquor and black liquor are charged in an amount such that the alkali charge is 200 kg of active alkali (NaOH) per ton of absolutely dry wood, and the wood:liquor ratio is 1:3.0.

The cook is heated by the supply of direct steam through the conduit 14 to the bottom of the digester. The steam supply is controlled by the valve 15 so that the heating to 170°C is effected within 30 minutes. During the cooking step de-gassing of air, turpentine, etc., takes place all the time in a normal manner through the conduit 16 and with de-gassing control by the valve 17.

The temperature in the top of the digester having reached 155°C, the first surge-boil is carried out. This is effected by opening the valve 13 for 5 minutes so that a substantial de-gassing takes place through the conduit 12. The surge-boil de-gassing is to be so substantial that at each surge-boil 0.5 - 5% of the total liquor amount is removed from the digester. The de-gassed liquor thereby removed comprises about 5 - 25% steam, the remainder being foam and liquor droplets.

The heating of the cook by direct steam continues during the surge-boil period in a normal manner.

The temperature in the digester having reached 170°C, the steam supply is interrupted by closing the valve 15.

After 5 minutes at 170°C the second surge-boil is effected by again opening the valve 13 for 5 minutes and simultaneously also charging steam by opening the valve 15. The steam is to be charged in an amount of the magnitude 0.1 - 0.5 ton steam/minute.

After completing the second surge-boil the valves (13) and (15) are again closed.

5 After another 80 minutes at 170°-175°C, the cooking is interrupted by taking in cooling liquor to the digester top for about 5 minutes; whereafter the digester is blown. Blowing time = 30 minutes.

10 The chlorine number of the pulp was 6.0 and the shive content when straining an average sample from the cook in a Wennberg-strainer with slit width 0.20 mm was 1.5%. For a cook in which the surge-boil technique was not utilized, the shive content was 7.0% at a chlorine number of 6.0.

15 I claim:

1. In a method of improving the homogeneity in periodic cooking of lignocellulosic material in a digester including a heating stage and having a heating system constructed in a manner to permit steam to be supplied directly to the bottom of the digester wherein at least one surge-boil step having a duration of from 10 minutes to 5 seconds is carried out, during the heating period of the cooking stage at a point of time when the chlorine number of the pulp is 30-20, by pressure reduction in the digester, said pressure reduction being obtained by carrying out at least one of the steps of (a) removing gas from the top of the digester and (b) supplying cooling liquid to the top of the digester, the improvement which consists in enhancing the surge-boil step by simultaneously with the pressure reduction directly supplying steam to the digester bottom in an amount of at least 0.1 ton steam/minute.

\* \* \* \* \*

30

35

40

45

50

55

60

65

UNITED STATES PATENT OFFICE  
CERTIFICATE OF CORRECTION

PATENT NO. : 3,907,631

DATED : September 23, 1975

INVENTOR(S) : Sture Olof Erik Backlund

It is certified that error appears in the above-identified patent and that said Letters Patent are hereby corrected as shown below:

[73] Assignee: SCA Projekt Aktiebolag

Signed and Sealed this

ninth Day of December 1975

[SEAL]

Attest:

RUTH C. MASON

*Attesting Officer*

C. MARSHALL DANN

*Commissioner of Patents and Trademarks*